

# United States Patent [19]

Harnisch et al.

[11] Patent Number: 4,812,379

[45] Date of Patent: Mar. 14, 1989

[54] ELECTROPHOTOGRAPHIC TONERS  
CONTAINING AN ADDITIVE  
REINFORCING THE CATIONIC CHARGE

[75] Inventors: Horst Harnisch, Much; Roderich Ruae, Leverkusen, both of Fed. Rep. of Germany

[73] Assignee: Bayer Aktiengesellschaft,  
Leverkusen, Fed. Rep. of Germany

[21] Appl. No.: 10,364

[22] Filed: Feb. 3, 1987

[30] Foreign Application Priority Data

Feb. 15, 1986 [DE] Fed. Rep. of Germany ..... 3604827

[51] Int. Cl.<sup>4</sup> ..... G03G 9/16

[52] U.S. Cl. ..... 430/110; 430/106.6

[58] Field of Search ..... 546/110; 544/357, 361;  
430/108, 110, 106.6

[56] References Cited

U.S. PATENT DOCUMENTS

4,680,245 7/1987 Suematsu et al. ..... 430/110  
4,686,166 8/1987 Kumagai et al. ..... 430/110

Primary Examiner—John L. Goodrow  
Attorney, Agent, or Firm—Sprung Horn Kramer & Woods

[57] ABSTRACT

Positively charged electrophotographic toners contain, in addition to conventional resin and pigment particles, an additive reinforcing the cationic charge, of the general formula



-continued



in which

R<sup>1</sup> and R<sup>2</sup> each represent hydrogen, chlorine, bromine, hydroxyl, C<sub>1</sub>-C<sub>4</sub>-alkoxy or carboxyl,  
A represents C<sub>1</sub>-C<sub>5</sub>-alkylene or —C<sub>6</sub>H<sub>4</sub>—CH<sub>2</sub>—(m or p),  
m represents 0 to 1,  
n represents 1 or 2  
K<sup>+</sup> represents



R<sup>3</sup> represents C<sub>1</sub>-C<sub>18</sub>-alkyl, carbamoyl-C<sub>1</sub>-C<sub>2</sub>-alkyl, C<sub>1</sub>-C<sub>4</sub>-alkoxycarbonyl-C<sub>1</sub>-C<sub>2</sub>-alkyl, benzyl, cyclohexyl or allyl,

R<sup>4</sup> represents C<sub>1</sub>-C<sub>4</sub>-alkyl or a single bond linked to D,

R<sup>5</sup> represents C<sub>1</sub>-C<sub>4</sub>-alkyl,

D represent —CH<sub>2</sub>—, —CH<sub>2</sub>—CO—, —CH<sub>2</sub>—CO—NH— or —CH<sub>2</sub>—CO—NH—CH<sub>2</sub>—

W represents



—CO— or a single bond,  
Z represents —CH<sub>2</sub>—,



—O—, —S—, —SO<sub>2</sub>— or a single bond and  
An<sup>+</sup> represents an anion.

4 Claims, No Drawings

ELECTROPHOTOGRAPHIC TONERS  
CONTAINING AN ADDITIVE REINFORCING THE  
CATIONIC CHARGE

The invention relates to positively charged electrophotographic toners which contain, in addition to conventional resin and pigment particles, an additive reinforcing the cationic charge, of the general formula



in which

R<sup>1</sup> and R<sup>2</sup> each represent hydrogen, chlorine, bromine, hydroxyl, C<sub>1</sub>-C<sub>4</sub>-alkoxy or carboxyl,

A represents C<sub>1</sub>-C<sub>5</sub>-alkylene or -C<sub>6</sub>H<sub>4</sub>-CH<sub>2</sub>- (m or p),

m represents 0 or 1

n represents 1 or 2

K<sup>+</sup> represents



R<sup>3</sup> represents C<sub>1</sub>-C<sub>18</sub>-alkyl, carbamoyl-C<sub>1</sub>-C<sub>2</sub>-alkyl, C<sub>1</sub>-C<sub>4</sub>-alkoxycarbonyl-C<sub>1</sub>-C<sub>2</sub>-alkyl, benzyl, cyclohexyl or allyl,

R<sup>4</sup> represents C<sub>1</sub>-C<sub>4</sub>-alkyl or a single bond linked to D,

R<sup>5</sup> represents C<sub>1</sub>-C<sub>4</sub>-alkyl,

D represents -CH<sub>2</sub>-, -CH<sub>2</sub>-CO-, -CH-



-CO- or a single bond,  
Z represents -CH<sub>2</sub>-,

10

15



-O-, -S-, -SO<sub>2</sub>- or a single bond and  
An<sup>(-)</sup> represents an anion,  
to the use of the compounds (I) in electrographic toners  
and to novel naphthalic acid imide derivatives.

20 R<sup>1</sup> and R<sup>2</sup> preferably denote hydrogen.  
C<sub>1</sub>-C<sub>5</sub>-alkylene radicals A can be straight-chain or  
branched. C<sub>2</sub>-C<sub>5</sub>-alkylene radicals and in particular the  
n-propylene radical are preferred.

Preferred alkyl radicals R<sup>3</sup> are C<sub>1</sub>-C<sub>6</sub>-alkyl radicals.  
Suitable anions are conventional anions such as halides, for example chloride, bromide and iodide, tetrafluoroborates and anions of alkylsulphonic and arylsulphonic acids, of alkylcarboxylic and arylcarboxylic acids, of alkylphosphoric and arylphosphoric acids and

30 of alkylphosphonic and arylphosphonic acids. Anions which reduce the water-solubility of the compounds (I) and at the same time increase their solubility in organic solvents such as dimethylformamide, acetone, chloroform or toluene are particularly suitable. The reduction of water-solubility can however also be achieved by increasing the size of the alkyl radical R<sup>3</sup>, i.e. by selecting it approximately in the range of C<sub>5</sub>-C<sub>16</sub>-alkyl. In this case more hydrophilic anions such as halides are also highly suitable.

40 The preferred water-solubility of the compounds (I) at 20° C. is below 3% by weight, in particular below 1% by weight. In addition to halides and tetrafluoroborates, particularly preferred anions are arylsulphonates such as benzenesulphonates, optionally substituted by C<sub>1</sub>-C<sub>12</sub>-alkyl or chlorine, C<sub>5</sub>-C<sub>18</sub>-alkylsulphonates, salts of C<sub>5</sub>-C<sub>18</sub>-alkylcarboxylic acids and salts of condensation products of formaldehyde and arylsulphonic acids and/or optionally sulphonated 4,4'-dihydroxydiphenylsulphone.

50 Preferred compounds of the formula (I) correspond to the formula



65

in which

A<sup>1</sup> represents C<sub>2</sub>-C<sub>5</sub>-alkylene,  
K<sup>1</sup> represents

<sup>2</sup>-CO-NH- or -CH<sub>2</sub>-CO-NH-CH<sub>2</sub>-  
W represents



R<sup>6</sup> represents C<sub>1</sub>-C<sub>16</sub>-alkyl, carbamoylmethyl or benzyl,

R<sup>7</sup> represents methyl or ethyl or a single bond linked to D,

R<sup>8</sup> represents methyl or ethyl,

W<sup>1</sup> represents



Z<sup>1</sup> represents —CH<sub>2</sub>—,



—O— or —SO<sub>2</sub>— and

X<sup>⊖</sup> represents an anion, and

D, m and n have the same meaning as in formula (I).

The compounds of the formula (I) can be prepared by known methods, for example by the method described in DE-A 3,535,496. The compounds themselves are mostly known.

Charge-reinforcing additives for electrophotographic toners, also referred to as charge-regulating substances, are already known. They are described, for example in U.S. Pat. Nos. 3,893,935, 3,944,493, 4,007,293, 4,079,014, 4,298,672, 4,338,390, 4,394,430 and 4,493,883.

Latent electrostatic image recordings are developed by inductive deposition of the toner on the electrostatic image. The charge-regulating substances reinforce the cationic charge of the toner. The image thereby becomes stronger and sharper.

Such charge-regulating substances must meet a variety of requirements.

1. Capability of developing the latent electrostatic image to a strongly coloured visible image.

2. Ready dispersibility in the toner composition and uniform dispersion on the image surface in order to produce a defect-free, sharp, homogeneous image.

3. Insensitivity to moisture.

4. High thermal stability.

5. Resistance to the hot mixture of lead oxide and a vinylidene fluoride/hexafluoropropylene copolymer resin (for example VITON® E-430 from Dupont) which can be used to fix the image with the aid of a hot roller. The coating composition must not turn black as a result of decomposition products.

6. Absence of toxicity.

The charge-regulating substances known from the abovementioned U.S. patents by no means meet all these requirements.

It has now been found, surprisingly, that the substances (I) are highly suitable as charge-regulating substances in toners. In comparison with the cationic phthalimide compounds known from U.S. Pat. No. 4,493,883, the compounds (I) produce a distinct increase in the colour strength of the developed image and an improvement in image sharpness. A further advantage

is the considerably improved pH stability, which allows the preparation both of the compounds and of the toner compositions without any problems.

The resins contained in the toners are known. They are thermoplastic and have a softening point between 50° and 130° C., preferably between 65° and 115° C. Examples of such resins are polystyrene, copolymers of styrene with an acrylate or methacrylate, copolymers of styrene with butadiene and/or acrylonitrile, polyacrylates and polymethacrylates, copolymers of an acrylate or methacrylate with vinyl chloride or vinyl acetate, polyvinyl chloride, copolymers of vinyl chloride with vinylidene chloride, copolymers of vinyl chloride with vinyl acetate, polyester resins (U.S. Pat. No. 3,590,000), epoxy resins, polyamides and polyurethanes.

In addition to the compounds (I) and the thermoplastic resins, the toners according to the invention contain known amounts of colouring materials and magnetically attractive material. The colouring material can consist of an organic dyestuff such as nigrosin, aniline blue, 2,9-dimethylquinacridone, C.I. Disperse Red 15 (=C.I. 60,710), C.I. Solvent Red 19 (=C.I. 26,050), C.I. Pigment Blue 15 (=C.I. 74,160), C.I. Pigment Blue 22 (=C.I. 69,810) and C.I. Solvent Yellow 16 (=C.I. 12,700), or an inorganic pigment such as carbon black, red lead, yellow lead oxide or chrome yellow. Generally, the amount of the colouring material present in the toners does not exceed about 15% by weight.

The magnetically attractive material can consist of, for example, iron, nickel, chromium oxide, iron oxide or a ferrite of the general formula MFe<sub>2</sub>O<sub>4</sub>, in which M represents a divalent metal such as iron, cobalt, zinc, nickel or manganese.

The preparation of the toners containing the compounds (I) is carried out by conventional methods, for example by melting the thermoplastic resin or a mixture of the thermoplastic resins, then finely dispersing one or more charge-regulating substances of the formula (I) and other additives, if used, in the molten resin, using the mixing and kneading machinery known for this purpose, then cooling the melt to a solid mass and finally grinding the solid mass to particles of the desired particle size. It is also possible to dissolve the thermoplastic resin and the compound (I) in a common solvent, incorporate the other additives into the solution and then spray-dry the liquid in a manner known per se or evaporate the solvent or solvents and grind the solid residue to particles of the desired particle size. In a modification of this method of preparation, the charge-regulating substance of the formula (I) is not dissolved but finely dispersed in the solution of the thermoplastic resin.

The toner composition obtained in this manner is then used, for example by analogy with U.S. Pat. No. 4,265,990, in a xerographic image-recording system. The photoreceptors employed for this purpose must be capable of becoming negatively charged. Examples are those likewise described in U.S. Pat. No. 4,265,990. They can contain, for example, the substances listed below in the charge-generating layer: 4-dimethylaminobenzylidenebenzhydrazide, polyvinylcarbazole, 2-benzylideneaminocarbazole, 2-nitrobenzylidene-p-bromoaniline, 2,4-diphenylquinazoline, 1,5-diphenyl-3-methylpyrazoline, 1,3,5-triphenylpyrazoline, charge-transfer complex from polyvinylcarbazole and trinitrofluorenone, 2-(4'-dimethylaminophenyl)-benzoxazole, selenium, tellurium, and arsenic triselenide.

The photoreceptors used can also additionally contain sensitizing dyes in the charge-generating layer.

colourless and dried in vacuo at 60° C. 444 g (97% of theory) of a compound of the formula



such as, for example, Bengal pink or eosine G. The photoreceptors can contain diamines in the charge-transporting layer, as are likewise mentioned in U.S. Pat. No. 4,265,990.

The compounds of the formula (II) are also a subject of the invention.

### EXAMPLE 1

282 g of naphthalic acid N-(3-dimethylaminopropyl)imide (1 mole) and 175.5 g of 4,4'-bis(chloroacetamido-phenyl)-methane (0.5 mole) are heated in 1330 g of polyglycol (mean molecular weight 400) at 100° C. for 3 hours, a clear viscous solution initially forming from which a colourless crystalline precipitate subsequently separates. After cooling to room temperature, the reaction mixture is diluted with 3.3 l of isopropanol with stirring, the crystalline precipitate is filtered off with suction, washed with isopropanol until the washings are

are obtained. The substance is virtually pure, as shown by thin-layer chromatography. 1 exhibits fluorescence quenching on the fluorescent silica gel plate.  $R_f$ : 0.3 (mobile phase: 45% by volume of butyl acetate, 33% by volume of glacial acetic acid, 9% by volume of formic acid and 13% by volume of water).

The compounds listed below are prepared in an analogous manner:



| Example | A                                                  | $\text{--K--}$                           | D                                             | W               |
|---------|----------------------------------------------------|------------------------------------------|-----------------------------------------------|-----------------|
| 2       |                                                    | $\text{--N}(\text{CH}_3)_2^+$            | $\text{--CH}_2\text{--CO--NH--}$              |                 |
| 3       |                                                    | $\text{--N}(\text{CH}_3)_2^+$            | $\text{--CH}_2\text{--CO--NH--}$              |                 |
| 4       | $\text{--CH}_2\text{--CH}_2\text{--}$              | $\text{--N}(\text{CH}_2\text{CH}_3)_2^+$ | $\text{--CH}_2\text{--CO--NH--}$              |                 |
| 5       | $\text{--CH}_2\text{--CH}_2\text{--CH}_2\text{--}$ | $\text{--N}(\text{CH}_3)_2^+$            | $\text{--CH}_2\text{--CO--NH--}$              |                 |
| 6       |                                                    | $\text{--N}(\text{CH}_3)_2^+$            | $\text{--CH}_2\text{--CO--NH--CH}_2\text{--}$ |                 |
| 7       | $\text{--CH}_2\text{--CH}_2\text{--}$              |                                          | $\text{--CH}_2\text{--}$                      | $\text{--CO--}$ |
| 8       | $\text{--CH}_3\text{--}(\text{CH}_2)_3\text{--}$   | $\text{--N}(\text{C}_2\text{H}_5)_2^+$   | $\text{--CH}_2\text{--}$                      |                 |

-continued

| Example | A                                                                                 | $\text{--K}^+$                                                                    | D                                   | W                                                                                   |
|---------|-----------------------------------------------------------------------------------|-----------------------------------------------------------------------------------|-------------------------------------|-------------------------------------------------------------------------------------|
| 9       | $-\text{CH}_2-\text{CH}_2-$                                                       |  | $-\text{CH}_2-\text{CO}-$           |  |
| 10      |  |  | $-\text{CH}_2-\text{CO}-\text{NH}-$ |   |

The compounds listed below are also prepared in an analogous manner:

are obtained, melting point 186°–188° C. The substance is virtually pure, as shown by thin-layer chromatogra-



| Example | S¹                               | S²                               |
|---------|----------------------------------|----------------------------------|
| 11      | Cl                               | H                                |
| 12      | Cl                               | Cl                               |
| 13      | $\text{CH}_3-\text{O}-$          | H                                |
| 14      | $\text{C}_2\text{H}_5-\text{O}-$ | H                                |
| 15      | $\text{CH}_3-\text{O}-$          | $\text{CH}_3-\text{O}-$          |
| 16      | $\text{C}_2\text{H}_5\text{O}-$  | $\text{C}_2\text{H}_5-\text{O}-$ |
| 17      | Br                               | H                                |
| 18      | Br                               | Br                               |
| 19      | COOH                             | H                                |
| 20      | COOH                             | COOH                             |

### EXAMPLE 21

282 g of naphthalic acid N-(3-dimethylaminopropyl)-imide are reacted with 175.5 g of 4,4'-bis(chloroacetamidophenyl)-methane in 1330 g of polyglycol at 100° C. for 3 hours in the same manner as described in Example 1, 600 ml of ethanol and 225 g of p-toluenesulphonic acid are added, the mixture is heated to boiling under reflux for 2 hours, and the colourless crystalline precipitate is filtered off with suction, washed with 800 ml of ethanol and dried in vacuo at 60° C.

366 g of a compound of the formula

phy.

The p-toluenesulphonates and benzenesulphonates of the compounds 2 to 20 are also prepared in an analogous manner.

### EXAMPLE 22

56.5 g (0.2 mole) of naphthalic acid N-(3-dimethylaminopropyl)-imide are suspended in 700 ml of toluene; 56 g of methyl p-toluenesulphonate are added with stirring, and stirring is continued at 60° C. for 1 hour. The colourless crystalline precipitate is filtered off with suction, washed with 150 ml of isopropanol and



Melting point 186–188° C.

9

dried in vacuo at 40° C. 87 g (93% of theory) of a compound of the formula

10  
are obtained. The substance is entirely pure, as shown by thin-layer chromatography. It melts at 220°–221° C. The substances listed below of the formula



are prepared in an analogous manner.

-continued

| Example | R <sup>1</sup> | R <sup>2</sup> | A                                  | K <sup>1</sup> Θ                                                                                                                       | X <sup>Θ</sup>  |
|---------|----------------|----------------|------------------------------------|----------------------------------------------------------------------------------------------------------------------------------------|-----------------|
| 33      | H              | H              | —(CH <sub>2</sub> ) <sub>3</sub> — | $  \begin{array}{c}  \text{CH}_3 \\    \oplus \\  -\text{N}—\text{C}_{16}\text{H}_{31}(\text{n}) \\    \\  \text{CH}_3  \end{array}  $ | Cl <sup>Θ</sup> |

10

**EXAMPLE 34**

15

282 g (1 mole) of naphthalic acid N-(3-dimethylaminopropyl)-imide are suspended in 21 acetonitrile, and the suspension is treated with 307 g (1 mole) of 1-bromohexadecane with stirring and heated to boiling 20 under reflux for 15 hours. The solution is filtered warm at 35° C. to remove small amounts of undissolved components. The filtrate is stirred with 2.5 l of acetone and cooled to -5° C. The crystalline precipitate is filtered off with suction, washed first with acetone then with 25 petroleum ether, and dried in vacuo at 30° C. 540 g (92% of theory) of a compound of the formula



are obtained.

### EXAMPLE 35

289 g (1.02 mole) of naphthalic acid N-(3-dimethylaminopropyl)-imide are suspended in 6.1 l of toluene and the suspension is treated dropwise with 138 g (1.09 mole) of dimethyl sulphate at 60° to 65° C. with stirring, and stirring is continued at 60° to 65° C. for 6 hours. After cooling to room temperature, the crystalline precipitate is filtered off with suction, washed with toluene and dried in vacuo at 50° C. 408 g (98% of theory) of a compound of the formula



are obtained.

408 g (1 mole) of the compound obtained (35 A) are dissolved in 4 l of water at room temperature and the solution is treated dropwise, with stirring, with 1 l of a 40% strength aqueous solution of a polycondensation product of sulphonated 4,4'-dihydroxydiphenylsulphone and formaldehyde. The crystalline precipitate is filtered off with suction, washed with water and dried in vacuo at 50° C. 685 g of a compound of the formula

15

20

25

(35)

are obtained.

$Q\Theta$ —equivalent of an anion obtained by condensing 4,4'-dihydriodiphenylsulphone, sulphuric acid and formaldehyde in the molar ratio 1:1:0.67.

#### APPLICATION EXAMPLE

2 percent by weight of the compound from Example 35 22, 6 percent by weight of carbon black and 92 percent by weight of a styrene/butadiene resin containing 89 percent by weight of styrene and 11 percent by weight of butadiene are melted together in an extruder at 100° C. and kneaded, and subsequently comminuted and ground until the particle diameter is smaller than 5 $\mu$ .

This toner composition is incorporated into a xerographic image recording system, such as that described in U.S. Pat. No. 4,265,990. For this purpose a MYLAR® substrate is provided with a polyvinylcarbazole layer which is charge-generating when illuminated and in which trigonal selenium is freely dispersed; this is overlaid with a transparent charge-transporting layer containing N,N'-diphenyl-N,N'-bis-(3-methylphenyl)-1,1'-bisphenyl-4,4'-diamine, dispersed in a MAKROLON® polycarbonate composition, as the charge-transporting molecule.

Microscopically sharp image recordings are obtained which in their sharpness are superior even to those produced according to U.S. Pat. No. 4,493,883, Example 1.

We claim:

## 1. Electrophotographic toners comprising an additive reinforcing the cationic charge, of the formula



-continued

5  
10

in which

R<sup>1</sup> and R<sup>2</sup> each represent hydrogen, chlorine, bromine, hydroxyl, C<sub>1</sub>-C<sub>4</sub>-alkoxy or carboxyl,  
A represents C<sub>1</sub>-C<sub>5</sub>-alkylene or —C<sub>6</sub>H<sub>4</sub>—CH<sub>2</sub>— (m 15 or p),  
m represents 0 or 1,

n represents 1 or 2

K<sup>⊕</sup> represents

20

in which  
A¹ represents C<sub>2</sub>-C<sub>5</sub>-alkylene,  
K¹⊕ represents



R<sup>3</sup> represents C<sub>1</sub>-C<sub>18</sub>-alkyl, carbamoyl-C<sub>1</sub>-C<sub>2</sub>-alkyl, C<sub>1</sub>-C<sub>4</sub>-alkoxycarbonyl-C<sub>1</sub>-C<sub>2</sub>-alkyl, benzyl, cyclohexyl or allyl,

R<sup>4</sup> represents C<sub>1</sub>-C<sub>4</sub>-alkyl or a single bond linked to D,

R<sup>5</sup> represents C<sub>1</sub>-C<sub>4</sub>-alkyl,

D represents —CH<sub>2</sub>—, —CH<sub>2</sub>—CO<sub>13</sub>—, —CH<sub>2</sub>—CO—NH— or —CH<sub>2</sub>—CO—NH—CH<sub>2</sub>—

W represents



30

R<sup>6</sup> represents C<sub>1</sub>-C<sub>16</sub>-alkyl, carbamoylmethyl or benzyl,

R<sup>7</sup> represents methyl or ethyl or a single bond linked to D,

R<sup>8</sup> represents methyl or ethyl,

W¹ represents



35

Z¹ represents —CH<sub>2</sub>—,

40

—O— or —SO<sub>2</sub>— andX<sup>⊖</sup> represents an anion, and

D, m and n having the meaning given in claim 1.

3. Electrophotographic toners according to claim 1, further comprising a magnetically attractable material.

4. A method of reinforcing the positive charge in electrophotographic toners comprising adding to the toner an additive reinforcing the cationic charge according to claim 1.

\* \* \* \* \*



—O—, —S—, —SO<sub>2</sub>— or a single bond and  
An<sup>⊖</sup> represents an anion, resin and pigment particles.

2. Electrophotographic toners according to claim 1, 55 wherein the additive reinforcing the cationic charge is of the formula

50

60

65

UNITED STATES PATENT AND TRADEMARK OFFICE  
CERTIFICATE OF CORRECTION

PATENT NO. : 4,812,379  
DATED : March 14, 1989

INVENTOR(S) : Horst Harnisch, et al

It is certified that error appears in the above-identified patent and that said Letters Patent is hereby corrected as shown below:

|                                  |                                                                                                  |
|----------------------------------|--------------------------------------------------------------------------------------------------|
| Title Page, Abstract,<br>line 12 | Delete "0 to 1" and substitute<br>--0 or 1--                                                     |
| Col. 2, line 25                  | Delete "C <sub>1</sub> -C <sub>6</sub> -" and substitute<br>--C <sub>1</sub> -C <sub>16</sub> -- |
| Col. 2, line 67                  | Delete "K <sup>1</sup> Θ" and substitute --K <sup>1</sup> ⊕--                                    |
| Col. 13, line 34                 | Delete "-CH <sub>2</sub> -CO13" and substitute<br>-- -CH <sub>2</sub> -CO --                     |
| Col. 14, line 50                 | Delete "having" and substitute<br>--have--                                                       |

Signed and Sealed this  
Twenty-seventh Day of February, 1990

*Attest:*

JEFFREY M. SAMUELS

*Attesting Officer*

*Acting Commissioner of Patents and Trademarks*